

## UNITED STATES PATENT OFFICE

2,031,046

PROCESS FOR THE PREVENTION OF THE  
BLEEDING ON WHITE ANIMAL FIBERSAlbert Landolt, Basel, Switzerland, assignor to  
the firm Society of Chemical Industry in Basle,  
Basel, SwitzerlandNo Drawing. Application June 17, 1931, Serial  
No. 545,145. In Switzerland June 20, 1930

7 Claims. (Cl. 8—12)

The present invention refers to a process for the prevention of the bleeding out of dyed textiles on white animal fibers, particularly wool, but also natural silks, in presence of aqueous solutions the pH of which is not greater than 7. It comprises the process herein referred to, and the wool treated according to the said process.

Dyed wool, as is well known, is washed and milled with aid of solutions having a more or less pronounced alkaline reaction. By this operation a more or less considerable amount of the dyestuff is very easily removed from the fiber, so that if dyed wool is intended to be washed or milled, the wool must from the start be dyed with dyestuffs fast to washing or milling. Formerly such dyestuffs were the after chroming dyestuffs. In recent times other classes of dyestuffs have been placed on the market the dyeings of which from an acid bath withstand washing and milling. Such dyestuffs are for example the products known in the trade as "Neolan" dyestuffs, "Lanasol" dyestuffs, cloth fast dyestuffs, "Fullacine" dyestuffs, etc.—"Neolan", "Lanasol" and "Fullacine" being registered trade marks.

However, the wool is not only treated with aid of solutions having an alkaline reaction. It can also be treated with solutions which are neutral or weakly acid, i. e. with solutions the pH of which is not greater than 7. In these operations (for example water-milling, boiling in presence of acids, or acid-milling) the dyestuffs remain better fixed on the fiber in general than in the case of the treatment with alkaline solutions. In the said operations, however, in which the pH of the solution used does not lie above 7, a stronger bleeding out on white wool is in general taking place than in the case where the solutions used are alkaline.

I have now found that the auxiliary agents for the textile industry which possess the capability of lowering or eliminating or retarding the affinity of animal fibers for dyestuffs, are in a remarkable degree adapted to increase the fastness to acid milling, water milling and acid boiling of wool dyed with dyestuffs which dye from an acid bath. They are particularly capable to prevent the bleeding out of the dyed wool on white wool milled or boiled along with it.

Such textile auxiliary agents, which are able to lower or eliminate or retard the affinity of animal fibers for dyestuffs, are to a great extent already described in the patent, technical and scientific literature on the subject. Among these there are particularly mentioned inter alia the condensation products of sulfur and phenol,

which probably correspond to the various brands known on the market under the registered name Katanol and Thiotan; further the products which are formed by condensation of aromatic sulfonic acids, such as naphthalene sulfonic acid, with alcohols (aliphatic, cyclic, aromatic-aliphatic alcohols),—such condensation products correspond to the various brands known on the market under the registered names "Nekal" and "Leonil"; the products which can be obtained by condensation of aromatic sulfonic acids with benzoin and, if necessary, by further condensation with alcohol; further sulfo ricinates, such as the "Prestabite" oils of the commerce; further synthetic tanning agents, such as the condensation products of formaldehyde with naphthalene sulfonic acids, etc.

Since the number of acid wool dyestuffs is considerable which bleed out in acid and water milling, or when boiled in an acid bath and, therefore, stain white wool milled or boiled along with the dyed wool, the present process constitutes a great technical advance.

The following examples illustrate the invention, the names "Kiton", "Neolan", "Katanol", "Thiotan", "Lanasol", "Fullacid", "Nekal", "Rhodamine", "Leonil", "Prestabite", "Tartrazine" mentioned therein being registered trade marks.

## Example 1

Wool is dyed as usual in an acid bath with 3 per cent. of acid blue RBF (Colour Index page 337), and then subjected to the following acid milling: The dyed wool mixed with 50 per cent. of white wool is milled for 4 hours in a milling bath containing per litre 1 gram of sulfuric acid, and 5 per cent. of the product obtained by condensing naphthalene- $\beta$ -sulfonic acids with benzoin and isopropyl alcohol (cf. Example 1 of Patent No. 1,833,245), calculated on the weight of the wool. Proportion of material to milling liquor 1:50. The white wool milled along with the dyed wool is not or only very slightly stained, whereas strong bleeding takes place without the addition of the mentioned product.

## Example 2

Wool is dyed as usual with 2 per cent. of "Kiton" fast orange G (Colour Index No. 27) and subjected, after having been mixed with white wool, to the following water milling: the milling is performed during 4 hours at 50° C. in a milling bath containing per litre 5 per cent. of the product obtained by condensing naphthalene- $\beta$ -sulfonic acids with benzoin and isopropyl alcohol

(cf. Example 1 of Patent No. 1,833,245), calculated on the weight of the wool. Proportion of material to milling liquor 1:50. In this manner the bleeding of the dyestuff used on white wool is prevented to a great extent, which is not the case without the addition.

#### Example 3

Wool is dyed with 3 per cent. of "Neolan" orange 10 GRE (Schultz 1932, vol. 2, page 154) in the manner usual for Neolan colors and the dyed material, which may be mixed with white wool, is subjected to the following acid milling: 1 litre of milling liquor contains 1 gram of sulfuric acid 15 and 5 per cent. of "Katanol" WL calculated on the weight of the wool. Milling is performed during 4 hours at 50° C. The dyestuff does not stain white wool, but strong bleeding takes place 20 without the addition of Katanol WL.

#### Example 4

Wool dyed with 3 per cent. of "Neolan" green B (Colour Index Supplement, page 46) is boiled along with white wool in an acid bath of the following composition: 1 litre of water, 1 gram of sulfuric acid and 10 per cent. of the product obtained by condensing naphthalene- $\beta$ -sulfonic acids with benzoin and isopropyl alcohol (cf. Example 1 of Patent No. 1,833,245), calculated on 25 the weight of the wool. The whole is boiled for 1/2 hour, after which time the dyestuff has stained the white wool quite considerably less than had the addition of the said product to the acid boiling bath not been made. The shade of the dyed 30 goods changes very much less with addition, than 35 without addition of the mentioned product.

#### Example 5

In a hot acid bath wool dyed with "Kiton" blue 40 A (Colour Index No. 714) bleeds very strongly on to white wool. This bleeding out can be prevented if 2 grams of "Katanol" W per litre of treating liquor are added to the boiling acid bath. Even 45 after boiling for one hour, white wool is not bled on when treated in this manner.

#### Example 6

A material dyed with Orange II (Colour Index No. 151) is subjected in the following manner, 50 in the presence of white wool, to an acid-milling:—The milling is carried out for 4 hours with 2 grams of sulfuric acid per litre, at a temperature of 50° C. In this operation white wool is very 55 strongly bled on by orange II. However, if 2 grams of "Thiotan" RS per litre are added to the acid-milling bath, white wool is scarcely bled on. In a similar manner behave other acid wool dyestuffs, such as: "Tartrazine", (Schultz 1931, 60 vol. 1, No. 737) "Alizarine" fast violet R, (Colour Index Supplement, page 26) "Lanasol" green G, (Schultz 1932, vol. 2, page 142) "Kiton" fast red 6BL, (Schultz 1932, vol. 2, page 138) and even 65 direct dyeing dyestuffs, such as direct fast scarlet WS (Colour Index Supplement, page 39).

#### Example 7

A dyeing made with 3 per cent. of "Fullacid" red G (Schultz 1932, vol. 2, page 111) is treated 70 for 4 hours at 50° C. with a milling liquor containing per litre water 2 grams of "Katanol" W. The wool dyed with "Fullacid" red G does not bleed on to white wool or silk milled along with it, which would be the case without the said 75 addition.

#### Example 8

Wool dyed with 3 per cent. of "Kiton" red G (Colour Index No. 31) is boiled together with white wool in a bath containing 4 per cent. of sulfuric acid, 10 per cent. of Glauber's salt and 2 5 grams per litre of the product obtained by condensing naphthalene- $\beta$ -sulfonic acids with benzoin and isopropyl alcohol (cf. Example 1 of Patent No. 1,833,245). A bleeding of the dyestuff on to white wool boiled along with the dyed wool 10 hardly takes place.

#### Example 9

Woollen material dyed with 3 per cent. of "Kiton" fast orange G (Colour Index No. 27) is 15 subjected to an acid milling according to Example 7 above, while adding 2 grams of "Nekal" BX (probably a butylated naphthalene sulfonic acid) per litre of milling liquor. By the said addition 20 the bleeding of the dyestuff on to white wool milled along with the dyed wool is prevented. In a similar manner behave the dyestuffs: "Kiton" red 6B (Colour Index No. 57), "Kiton" red S (Colour Index No. 54), "Kiton" fast red R (Colour Index, page 357), acid "Rhodamine" 3R (Colour Index, page 337), acid violet 6BN (Colour Index No. 717), "Kiton" pure blue V (Colour Index No. 672 cf. Supplement page 44), benzyl green B (Colour Index No. 667), etc.

#### Example 10

The so-called water-milling, as described in Example 8, is carried out with woollen material dyed with 3 per cent. of brilliant "Kiton" red B (Colour Index No. 748). The milling liquor contains 2 grams of "Leonil" S (probably an alkylated naphthalene sulfonic acid) per litre. The dyestuff which, without this addition, bleeds strongly on white wool, leaves the same almost pure white.

#### Example 11

The bleeding out of the dyeing made with benzyl violet 5BN, (Colour Index No. 698) in an acid boiling bath according to Example 12, can be 45 prevented by adding 2 grams per litre of the condensation product of naphthalene sulfonic acid and formaldehyde. It is to be noted that not only the white wool boiled along with the dyed material, but also white cotton which may be present, 50 were protected against the bleeding on.

#### Example 12

The acid milling described in Example 7 is carried out with dyeings of 3 per cent. (calculated 55 on the weight of the wool) of "Kiton" blue A (Colour Index No. 714). An addition of 2 grams per litre of the condensation product of naphthalene sulfonic acid and formaldehyde prevents the bleeding out of the dyestuff on to white wool and 60 white cotton.

#### Example 13

The water-milling described in Example 8 is carried out with a woollen material dyed with 2 65 per cent. of brilliant "Kiton" red B (Colour Index No. 748). As an addition to the milling liquor, 2 grams per litre of the condensation product of naphthalene sulfonic acid and formaldehyde are used. The white wool simultaneously 70 milled, by this addition, has been protected against being bled on.

The quantity of the various auxiliary agents to be added may vary within wide limits.

The improvement of the fastness to acid mill- 75

ing, water milling and acid boiling is also manifest, if the wool to be dyed is already treated in the dyeing bath with the said additions, and then carrying out the mentioned fastness tests without further additions.

5 What I claim is:—

1. Process for the prevention of the bleeding of dyed wool onto undyed wool in the simultaneous milling of dyed wool and undyed wool in an aqueous solution having a pH-value not greater than 7, consisting in adding to the solution a textile auxiliary obtained by causing a compound selected from a group of products consisting of alcohols and aldehydes to react with a naphthalene monosulfonic acid.
- 10 2. Process for the prevention of the bleeding of dyed wool onto undyed wool in the simultaneous milling of dyed wool and undyed wool in an aqueous solution having a pH-value not greater than 7, consisting in adding to the solution a textile auxiliary obtained by causing a compound selected from a group of products consisting of alcohols and aldehydes to react with a naphthalene monosulfonic acid.
- 15 3. Process for the prevention of the bleeding of dyed wool onto undyed wool in the simultaneous acid milling of dyed wool and undyed wool in an aqueous solution having a pH-value smaller than 7, consisting in adding to the solution a textile auxiliary obtained by causing a compound selected from a group of products consisting of alcohols and aldehydes to react with a naphthalene sulfonic acid.

4. Process for the prevention of the bleeding of dyed wool onto undyed wool in the simultaneous acid milling of dyed wool and undyed wool in an aqueous solution having a pH-value smaller than 7, consisting in adding to the solution a textile auxiliary obtained by causing a compound selected from a group of products consisting of alcohols and aldehydes to react with a naphthalene monosulfonic acid.

5 5. Process for the prevention of the bleeding of dyed wool onto undyed wool in the simultaneous acid milling of dyed wool and undyed wool in an aqueous solution having a pH-value smaller than 7, consisting in adding to the milling bath a condensation product from formaldehyde and a naphthalene sulfonic acid.

10 6. Process for the prevention of the bleeding of dyed wool onto undyed wool in the simultaneous acid milling of dyed wool and undyed wool in an aqueous solution having a pH-value smaller than 7, consisting in adding to the milling bath a condensation product from benzoin and a naphthalene sulfonic acid.

15 7. Process for the prevention of the bleeding of dyed wool onto undyed wool in the simultaneous acid milling of dyed wool, and undyed wool in an aqueous solution having a pH-value smaller than 7, consisting in adding to the milling bath a condensation product from butyl alcohol and a naphthalene sulfonic acid.

20 25 30 ALBERT LANDOLT.